# EUROPEAN PATENT SPECIFICATION

(11) **EP 1 829 984 B1**
(45) Date of publication and mention of the grant of the patent: **17.10.2012**
(21) Application number: 07250856.7
(22) Date of filing: 01.03.2007
(51) Int. Cl.: C23C 4/12, C23C 4/10, C23C 28/00, C23C 30/00

(54) **Process for making a high density thermal barrier coating**
Verfahren zum Herstellen von einer hochdichten Wärmedämmbeschichtung
Procédé de fabrication d'un revêtement de barrière thermique à forte densité

(30) Priority: 01.03.2006 US 366900
(43) Date of publication of application: 05.09.2007
(73) Proprietor: United Technologies Corporation, Hartford, CT 06101 (US)
(72) Inventor: Frost, Aaron T., San Antonio, TX 78251 (US); Quinones, Jose, San Antonio, TX 78230 (US)
(74) Representative: Leckey, David Herbert

(56) References cited:
- EP-A2- 0 916 744
- JP-A- 2005 105 417
- US-A- 4 457 948
- US-A- 5 073 433
- US-A- 5 705 231
- US-A- 6 132 175
- US-A1- 2002 119 338

## Description

### FIELD OF USE

The present disclosure relates to thermal barrier coatings and, more particularly, to high density thermal barrier coatings.

### BACKGROUND OF THE INVENTION

Air plasma sprayed thermal barrier coatings (hereinafter "APS TBCs") are well known, having been used for several decades. They are typically formed from ceramic materials capable of withstanding high temperatures and are applied to metal articles to inhibit the flow of heat into these articles. It has long been recognized that if the surface of a metal article which is exposed to a high temperature environment is coated with an appropriate refractory ceramic material, then the rate at which heat passes into and through the metal article is reduced, thereby extending its applicable service temperature range, service longevity, or both, and reducing the article's future repair costs.

Prior art APS TBCs are typically formed from powdered metal oxides such as well known compositions of yttria stabilized zirconia (YSZ). These TBCs are formed by heating a gas-propelled spray of the powdered oxide material using a plasma-spray torch, such as a DC plasma-spray torch, to a temperature at which the oxide powder particles become momentarily molten. The spray of the molten oxide particles is then directed onto a receiving metal surface or substrate, such as the surface of an article formed from a high temperature Ti-based, Ni-based, or Co-based superalloy, thereby forming a single layer of the TBC. In order to make TBCs having the necessary thicknesses, the process is repeated so as to deposit a plurality of individual layers on the surface of interest. Typical overall thicknesses of finished TBCs are generally no greater than 0.1 inches.

One well recognized problem in the use of prior art TBC coatings, particularly on articles routinely cycled from ambient conditions up to extremely high temperatures such as those used in gas turbines, is that the exposure of TBCs to the very intense heat and rapid temperature changes associated with high velocity combustion gases can cause their failure by spallation, or spalling of the TBC from the surfaces of the metal articles which they are designed to protect, possibly due to thermal fatigue. Susceptibility to spallation in cyclic thermal environments is primarily due to the existence of horizontal cracking or in-plane (of the TBC) cracking. Horizontal cracks are known particularly to increase the susceptibility of a TBC to spallation because in-plane stresses, such as in-plane stresses created during the TBC deposition process or in service, can cause such horizontal cracks to propagate and grow.

It is known that the spallation resistance of TBCs in such environments can be improved by modifying certain characteristics of the coatings. For example, it is known that the performance of yttria stabilized zirconia (YSZ) TBCs is enhanced in cyclic thermal environments by developing a predominance of cracks normal to the TBC/metal article interface (i.e. vertical cracks) and a minimum of cracks parallel to such interface (i.e. horizontal cracks). Referring to another example in a microphotograph of FIG. 1, U.S. Patent No. 5,073,433 issued to Taylor teaches that the existence of homogeneously dispersed vertical macrocracking with a controlled amount of horizontal cracking within a TBC reduces the tendency for spalling within the coating, and thus increases the thermal fatigue resistance. Referring to yet another example in a microphotograph of FIG. 2, U.S. Patent No. 5,830,586 issued to Gray that the extending the directional solidification of continuous columnar grains in at least one layer of a TBC promotes a coherent, continuous columnar grain microstructure and reduces the tendency for spalling within the coating, and thus increases the thermal fatigue resistance. However, neither Taylor nor Gray considers improving the density and porosity as well, which allow oxygen to permeate the bond coat and cause spallation.

Consequently, there exists a need for a high density thermal barrier coating that possesses a density, cracking density and porosity sufficient to reduce spallation.

EP 0916744 discloses a YSZ abrasive blade tip coating prepared from a powder having an average equivalent spherical diameter of less than 40µm and a density of above about 90% of theoretical density.

US 5,705,231 discloses a segmented abradable ceramic coating system having superior abradability and erosion resistance.

US 4,457,948 discloses a plasma flame sprayed ceramic thermal barrier coating that is treated to improve resistance to damage from thermal cycling.

### SUMMARY OF THE INVENTION

In accordance with the present invention, there is provided a process for coating an article as claimed in claim 1.

The details of one or more embodiments of the invention are set forth in the accompanying drawings and the description below. Other features and advantages of the invention will be apparent from the description and drawings, and from the claims.

### BRIEF DESCRIPTION OF THE DRAWINGS

FIG. 1 is a microphotograph of a thermal barrier coating of the prior art;
FIG. 2 is a microphotograph of a thermal barrier coating of the prior art;
FIG. 3 is a flowchart representing a process in accordance with the present invention;.
FIG. 4 is a microphotograph of a 7EA First Bucket part no. GTD-111 produced by the General Electric Company coated with a non-heated treated yttria stabilized zirconia thermal barrier coating; and
FIG. 5 is a microphotograph of a 501F First Stage Blade produced by Siemens-Westinghouse coated with a heat-treated yttria stabilized zirconia thermal barrier coating.

Like reference numbers and designations in the various drawings indicate like elements.

### DETAILED DESCRIPTION

Generally, the high density thermal barrier coatings deposited in the process of the present invention exhibit over an aggregate coating area an average density value of between about 95% to 100%, an average porosity of between no more than about 5% and 0% an average cracking density of between about 1 crack to 20 cracks per linear inch (0.4 to 7.9 cracks per cm) of the thermal barrier coating. The high density thermal barrier coatings ideally exhibit a density of no less than about 98%, a corresponding porosity of no more than about 3% and a cracking density of no more than about 20 cracks per linear inch (7.9 cracks per cm) of the thermal barrier coating. While a certain amount of cracking density is good for thermal fatigue, a cracking density of greater than 20 cracks per linear inch (7.9 cracks per cm) allows oxygen to permeate the bond coat, oxidize the bond coat material and induce spallation. By increasing the coating density and reducing the amount of vertically oriented microcracks, both thermal fatigue and spallation are reduced, which actually extends the service life of the turbine engine component.

Referring now to FIG. 3, a flowchart representing the processes of the present invention is shown. An article may be provided and may be coated with a bond coat material at step 10. The bond coat material may comprise a McrAlY material. MCrAlY refers to known metal coating systems in which M denotes nickel, cobalt, iron, platinum or mixtures thereof; Cr denotes chromium; Al denotes aluminum; and Y denotes yttrium. MCrAlY materials are often known as overlay coatings because they are applied in a predetermined composition and do not interact significantly with the substrate during the deposition process. For.some non-limiting examples of MCrAlY materials see U.S. Pat. No. 3,528,861 which describes a FeCrAlY coating as does U.S. Pat. No. 3,542,530. In addition, U.S. Pat. No. 3,649,225 describes a composite coating in which a layer of chromium is applied to a substrate prior to the deposition of a MCrAlY coating. U.S. Pat. No. 3,676,085 describes a CoCrAlY overlay coating while U.S. Pat. No. 3,754,903 describes a NiCoCrAlY overlay coating having particularly high ductility. U.S. Pat. No. 4,078,922 describes a cobalt base structural alloy which derives improved oxidation resistance by virtue of the presence of a combination of hafnium and yttrium. A preferred MCrAlY bond coat composition is described in U.S. Pat. No. Re. 32,121, as having a general formula of MCrAlYHfSi and a weight percent compositional range of 5-40 Cr, 8-35 Al, 0.1-2.0 Y, 0.1-7 Si, 0.1-2.0 Hf, balance selected from the group consisting of Ni, Co, Fe and mixtures thereof. See also U.S. Pat. No. 3,928,026 and U.S. Pat. No. 4,585,481.

The bond coat material may also comprise Al, PtAl and the like, that are often known in the art as diffusion coatings. In addition, the bond coat material may also comprise Al, PtAl, MCrAlY as described above, and the like, that are often known in the art as cathodic arc coatings.

These bond coat materials may be applied by any method capable of producing a dense, uniform, adherent coating of the desired composition, such as, but not limited to, an overlay bond coat, diffusion bond coat, cathodic arc bond coat, etc. Such techniques may include, but are not limited to, diffusion processes (e.g., inward, outward, etc.), low pressure plasma-spray, air plasma-spray, sputtering, cathodic arc, electron beam physical vapor deposition, high velocity plasma spray techniques (e.g., HVOF, HVAF), combustion processes, wire spray techniques, laser beam cladding, electron beam cladding, etc. The bond coat materials may be applied to any suitable thickness for the purpose of the intended application as will be recognized by one of ordinary skill in the art.

After applying the bond coat layer to the article at step 10, the article may be coated with a thermal barrier composition (hereinafter "TBC composition") at a step 12 of FIG. 3. The article may comprise any part that is typically coated with a thermal barrier compound and, in particular, may comprise a part used in turbomachinery applications such as, but not limited to, any part having an airfoil, any part having a seal, including blades, vanes, stators, mid-turbine frame, fans, compressors, turbine casings, seals, plates, rings, combustor panels, combustor chambers, combustor bulkhead shields, disk side plates, fuel nozzle guides and the like. The article may comprise a nickel based superalloy, a cobalt based superalloy, a ferrous alloy such as steel, a titanium alloy, a copper alloy and combinations thereof.

The TBC composition may comprise a ceramic based compound for use with turbomachinery applications as known to one of ordinary skill in the art. Representative thermal barrier compounds include, but are not limited to, any stabilized zirconate, any stabilized hafnate, combinations comprising at least one of the foregoing compounds, and the like, for example, yttria stabilized zirconia, calcia stabilized zirconia, magnesia stabilized zirconia, yttria stabilized hafnia, calcia stabilized hafnia and magnesia stabilized hafnia. Preferably, yttria stabilized zirconia may be employed. Yttria stabilized zirconia is commercially available as 7YSZ^{®}. To achieve the desired properties, for example, aforementioned density, cracking density and porosity values, the TBC composition comprises a powder having a fine particle size distribution of no less than about 8 µm (microns) and no more than about 88 µm (microns). For example, the TBC composition may be a powdered yttria stabilized zirconia having a particle size distribution of no less than about 8 µm (microns) and no more than about 88 µm (microns).

The thermal barrier coatings are applied using the techniques of, plasma spray processes, low pressure plasma-spray, air plasma-spray, sputtering, cathodic arc, electron beam physical vapor deposition, high velocity plasma spray techniques (e.g., HVOF; HVAF), combustion processes, wire spray techniques, laser beam cladding, electron beam cladding, combinations comprising at least one of the foregoing techniques.

To achieve the desired density, cracking density and porosity properties the TBC composition may be applied using air plasma spray processes known to one of ordinary skill in the art. Preferably, the air plasma spray process is performed using an internally injected powder feeding mechanism such that the powdered TBC composition may feed directly into the plume of the plasma flame as the powder is being deposited. The air plasma spray apparatus may be operated at a current of between about 600 and 1000 amps to achieve the desired plasma flame temperature. Suitable internally injected powder feeding plasma spray apparatus include, but are not limited to, the Praxair SG-100 plasma spray gun, commercially available from Praxair, Inc. of Danbury, Connecticut.

This air plasma spray deposition technique ensures the powdered TBC composition may pass through the hottest part of the plasma flame and melt completely. Preferably, the plasma spray gun of the plasma spray apparatus may be positioned at between about 2 inches to 8 inches (5.1 to 20.3 cm) away from the surface of the article being coated. This distance ensures the melted TBC composition may be deposited upon the article as quickly as possible, thus preventing the melted TBC composition from absorbing an amount of oxygen sufficient to affect the resultant TBC coating properties. To further ensure the melted TBC composition may be deposited upon the article the plasma spray apparatus may employ an arc gas mixture composed of helium and argon in a ratio of between about 3:1 to 1:3 depending upon the operating conditions. As understood by one of.ordinary skill in the art helium gas is lighter than argon and moves more quickly, which actually causes the melted TBC composition particles to travel more quickly. Again, the melted TBC composition particles' increased velocity further ensure the melted TBC composition does not absorb an amount of oxygen sufficient to affect the resultant TBC coating properties.

After applying the TBC composition, the article may be heat treated at a step 14 of FIG. 3 to form the thermal barrier composition coating layer (hereinafter "TBC coating") at a step 16 of FIG. 3. The article may be heat treated under a vacuum of about 1x10⁻³ torr to 1x10⁻⁶ torr (133 to 0.13 mPa) at a temperature range of about 1,800°F to 2,200°F (982°C to 1204°C) for a time period of about 2 hours to 4 hours, or a temperature of about 1,800°F (982°C) for about 4 hours, preferably at a temperature of about 2,175°F (1191°C) for about 2 hours, and most preferably at a temperature of about 2,050°F (1121°C) for about 2 hours. The temperature and amount of time heat may be applied is dependent upon the composition of the substrate of the article as is recognized by one of ordinary skill in the art. Suitable vacuum furnaces for use herein include any vacuum furnaces known to one of ordinary skill in the art.

Referring now to FIG. 4, a microphotograph of a 7EA First Bucket, part number GTD-111 manufactured by the General Electric Company, is shown. The 7EA First Bucket part was coated in accordance with prior art processes, that is, the thermal barrier coating composition being applied was a coarse powder, a mixture of Ar and H gases were employed and the coatings were applied under conventional process conditions using a conventional plasma spray technique. The 7EA First Bucket part (hereinafter "7EA part") was coated with a metallic bond coat and a thermal barrier coating of yttria stabilized zirconia having a particle size distribution of - 200 mesh to 400 mesh (37 to 74 µm (microns). The yttria stabilized zirconia was applied using an internal powder injection plasma spray gun at a distance of 130 millimeters (5.12 inches), at a current of 600 amps and an arc gas flow rate of 46 liters per minute of Ar and 14 liters per minute of H. The coated 7EA part was then examined and determined to possess over an aggregate coating area an aggregate density of 90%, an aggregate porosity of 12.2% and an aggregate cracking density of 0 cracks per 2.04 µm (inch).

Referring now to FIG. 5, a microphotograph of a 501F First Stage Blade manufactured by Siemens-Westinghouse is shown. The 501F First Stage Blade part was coated utilizing a method and coating composition of the present invention. The 501F First Stage Blade part (hereinafter "501F part") was coated with a metallic bond coat and a thermal barrier coating of yttria stabilized zirconia having a particle size distribution of -325 mesh (less than 44 µm (microns). The yttria stabilized zirconia was applied under a vacuum of 1x10⁻³ torr to 1x10⁻⁶ torr (133 to 0.13 mPa) using an internal powder injection plasma spray gun at a distance of 102 millimeters (4 inches), at a current of 1000 amps and an arc gas flow rate of 50 standard cubic feet per hour (24 liters per minute) of Ar and 100 standard cubic feet per hour (47 liters per minute) of He. The 501F part having the TBC layer was then heat treated at a temperature of 2,050°F (1121°C) for a period of 2 hours. The coated 501F part was then examined and determined to possess over an aggregate coating area an aggregate density of 99.1%, an aggregate porosity of 1% and an aggregate cracking density of 6.66 cracks per 2.54 µm (inch).

When comparing the results shown in FIGS. 4 and 5, the TBC of FIG. 5 applied using a method of the present invention exhibit overall improved properties than the TBC of FIG. 4 applied using a conventional method of the prior art. The TBC of FIG. 4 exhibits a porosity of 12.1% that will permit an oxygen source, e.g., the atmosphere, to infiltrate and permeate the TBC coating. The TBC coating of FIG. 4 will spall and fall off the 7EA part much earlier than anticipated during its useful service life. On the other hand, the TBC coating of FIG. 5 exhibits an aggregate porosity of 1% which suggests the average porosity of the TBC coating may be in a range of 98%. to 100% at any given location. This porosity value ensures an oxygen source will not infiltrate and permeate the TBC coating as readily as the TBC shown in FIG. 4. As a result, the 501F part may be in service for a greater period of time, undergo less maintenance due to TBC related problems and incur fewer maintenance related costs.

The process of the present invention provides many advantages over prior art processes. The resultant TBC coating possesses a cracking density of typically zero. Prior art TBC coatings exhibit 20 to 200 cracks per linear inch (7.9 to 79 cracks per cm) of coating, and typically exhibit 75 cracks per linear inch (30 cracks per cm) of coating. As a direct result, prior art TBC coatings also fail to exhibit a density greater than 98% due to the greater number of cracks per linear square inch of coating. In contrast, the TBC coatings deposited in the process of the present invention exhibit a density of no less than about 98%, which corresponds to a porosity of no more than about 3%, preferably no more than about 2%, and most preferably no more than about 1%.

It is to be understood that the invention is not limited to the illustrations described and shown herein, which are deemed to be merely illustrative of the best modes of carrying out the invention, and which are susceptible to modification of form, size, arrangement of parts, and details of operation. The invention rather is intended to encompass all such modifications which are within its scope as defined by the claims.

## Claims

1. A process for coating an article, comprising:
applying (10) a bond coat layer onto at least one surface of an article; and
applying (12) upon said bond coat layer a thermal barrier coating composition comprising a particle size distribution of no less than 8 microns and no more than 88 microns;
heat treating (14,16) said thermal barrier coating composition at a temperature of between 1,800°F to 2,200°F (982°C to 1204°C) for 2 hours to 4 hours at a pressure of 1x10⁻³ torr to 1x10⁻⁶ torr (133 to 0.13 mPa) to form a thermal barrier coating layer comprising a cracking density of 1 crack to 20 cracks per linear inch (0.4 to 7.9 cracks per cm) of said thermal barrier coating, an average porosity of between no more than 5 percent and 0 percent, and an average density of between 95 percent and 100 percent; and wherein
the application of said thermal barrier coating composition comprises a process selected from the group consisting of plasma spray processes, low pressure plasma-spray processes, air plasma-spray processes, sputtering processes, cathodic arc processes, electron beam physical vapor deposition processes, high velocity plasma spray processes, combustion processes, wire spray processes, laser beam cladding processes, electron beam cladding processes or a combination comprising at least one of these processes.

2. The process of claim 1, wherein the heat treating step (14) comprises heat treating said thermal barrier coating composition under said vacuum at a temperature of 2,175°F (1191°C) for 2 hours.

3. The process of claim 1, wherein the heat treatment step (14) comprises heat treating said thermal barrier coating composition under said vacuum at a temperature of 2,050°F (1121°C) for 2 hours.

4. The process of claim 1, wherein the heat treating step (14) comprises heat treating said thermal barrier coating composition under said vacuum at a temperature of 1,800°F (982ºC) for 4 hours.

5. The process of claim 1, wherein the heat treating step (14) comprises heat treating said thermal barrier coating composition under said vacuum at a temperature of 2,100°F (1149°C) for 4 hours.

6. The process of any preceding claim, wherein the application step (10) of said bond coat layer comprises a process selected from the group consisting of diffusion processes, plasma spray processes, low pressure plasma-spray processes, air plasma-spray processes, sputtering processes, cathodic arc processes, physical vapor deposition processes, electron beam physical vapor deposition processes, high velocity plasma spray processes, combustion processes, wire spray processes, laser beam cladding processes and electron beam cladding processes.

7. The process of any preceding claim, wherein the application step (12) of said thermal barrier coating composition comprises applying said thermal barrier coating composition using a plasma spray process.

8. The process of claim 7, wherein the application step (12) said thermal barrier coating composition comprises using an arc gas comprising helium and argon present in a ratio of 3:1 to 1:3.

9. The process of claim 7 or 8, wherein the application step of said thermal barrier coating composition comprises using an internal powder injection plasma spray gun.

10. The process of claim 9, further comprising operating said internal powder injection plasma spray gun at a current of between 600 to 1000 amps.

11. The process of claim 9 or 10, further comprising operating said internal powder injection plasma spray gun at a distance of 2 inches to 8 inches (5.1 to 20.3 cm) from said at least one surface of said article.

12. The process of any preceding claim, wherein said thermal barrier coating composition comprises a powdered ceramic material selected from the group consisting of yttria stabilized zirconia, calcia stabilized zirconia, magnesia stabilized zirconia, yttria stabilized hafnia, calcia stabilized hafnia and magnesia stabilized hafnia.

13. The process of any of claim 1 to 11, wherein said thermal barrier coating composition comprises a yttria stabilized zirconia powder.

## Patentansprüche

1. Verfahren zum Beschichten eines Gegenstands, aufweisend:
Aufbringen (10) einer Haftbeschichtungsschicht auf wenigstens eine Oberfläche eines Gegenstands; und
Aufbringen (12) auf die Haftbeschichtungsschicht einer Wärmedämmbeschichtungszusammansetzung, die eine Teilchengrößenverteilung von weniger als 8 Mikrometer und nicht mehr als 88 Mikrometer aufweist;
Wärmebehandeln (14, 16) der Wärmedämmbeschichtungzusammensetzung bei einer Temperatur zwischen 1800° F bis 2200° F (982° C bis 1204° C) für 2 Stunden bis 4 Stunden bei einem Druck von 1x10⁻³ Torr bis 1x10⁻⁶ Torr (133 bis 0,13 mPa), um eine Wärmedämmbeschichtungsschicht zu bilden, die aufweist eine Rissdichte von 1 Riss bis 20 Rissen pro Längen-Inch (0,4 bis 7,9 Risse pro cm) der Wärmedämmbeschichtung, eine durchschnittliche Porosität von zwischen nicht mehr als 5 Prozent und 0 Prozent, und eine durchschnittliche Dichte von zwischen 95 Prozent und 100 Prozent; und wobei
das Auftragen der Wärmedämmbeschichtungszusammensetzung ein Verfahren aufweist, welches ausgewählt ist aus der Gruppe, die besteht aus: Plasma-Sprühverfahren, Niederdruckplasma-Sprühverfahren, Luftplasma-Sprühverfahren, Sputter-Verfahren, physikalische Gasphasenabscheidungsverfahren mit Elektronenstrahl, Hochgeschwindigkeitsplasma-Sprühverfahren, Feuerungsverfahren, Draht-Sprühverfahren. Laserstrahlplattierungsverfahren, Elektronenstrahlplattierungsverfahren oder eine Kombination aufweisend wenigstens einen dieser Verfahren.

2. Verfahren gemäß Anspruch 1, wobei der Wärmebehandlungsschritt (14) Wärmebehandeln der Wärmedämmbeschichtungszusammensetzung unter dem Vakuum bei einer Temperatur von 2175° F (1191 °C) für 2 Stunden aufweist.

3. Verfahren gemäß Anspruch 1, wobei der Wärmebehandlungsschritt (14) Wärmebehandeln der Wärmedammbeschichtungszusammensetzung unter dem Vakuum bei einer Temperatur von 2050° F (1121° C) für 2 Stunden aufweist.

4. Verfahren gemäß Anspruch 1, wobei der Wärmebehandlungsschritt (14) Wärmebehandeln der Wärmedämmbeschichtungszusammensetzung unter dem Vakuum bei einer Temperatur von 1800° F (982° C) für 4 Stunden aufweist.

5. Verfahren gemäß Anspruch 1, wobei der Wärmebehandlungsschritt (14) Wärmebehandeln der Wärmedämmbeschichtungszusammensetzung unter dem Vakuum bei einer Temperatur von 2100° F (1149° C) für 4 Stunden aufweist.

6. Verfahren gemäß einem der vorhergehenden Ansprüche, wobei der Aufbringungsschritt (10) der Haftbeschichtungsschicht ein Verfahren aufweist, welches ausgewählt ist aus der Gruppe, die besteht aus: Diffusionsverfahren, Plasma-Sprühverfahren, Niederdruckplasma-Sprühverfahren, Luftplasma-Sprühverfahren, Sputter-Verfahren, Kathodenlichtbogenverfahren, physikalische Gasphasenabscheidungsverfahren, physikalische Gasphasenabscheidungsverfahren mit Elektronenstrahl, Hochgeschwindigkeitsplasma-Sprühverfahren, Feuerungsverfahren, Draht-Sprühverfahren, Laserstrahlplattierungsverfahren und Elektronenstrahlplattierungsverfahren.

7. Verfahren gemäß einem der vorhergehenden Ansprüche, wobei der Aufbringungsschritt (12) der Wärmedämmbeschichtungszusammensetzung Aufbringen der Wärmedämmbeschichtungszusammensetzung unter Verwendung eines Plasma-Sprühverfahrens aufweist.

8. Verfahren gemäß Anspruch 7, wobei der Aufbringungsschritt (12) der Wärmedämmbeschichtungszusammensetzung Verwenden eines Lichtbogengases aufweist, welches Helium und Argon in einem Verhältnis von 3:1 bis 1:3 aufweist.

9. Verfahren gemäß Anspruch 7 oder 8, wobei der Aufbringungsschritt der WArmedämmbeschichtungszusammensetzung Verwenden einer Plasmasprühkanone mit interner Pulvereinspritzung aufweist.

10. Verfahren gemäß Anspruch 9, weiter aufweisend Betreiben der Plasmasprühkanone mit interner Pulvereinspritzung bei einem Strom zwischen 600 bis 1000 Ampere.

11. Verfahren gemäß Anspruch 9 oder 10, weiter aufweisend Betreiben der Plasmasprühkanone mit interner Pulvereinspritzung bei einem Abstand von 2 inch bis 8 inch (5,1 bis 20,3 cm) von der wenigstens einen Oberfläche des Gegenstandes.

12. Verfahren gemäß einem der vorhergehenden Ansprüche, wobei die Wärmedämmbeschichtungszusammensetzung ein pulverisiertes Keramikmaterial aufweist, welches ausgewählt ist aus der Gruppe, die besteht aus: Yttrium-stabilisiertem Zirkonium, Calcium-stabilisiertem Zirkonium, Magnesium-stabilisiertem Zirkonium, Yttrium-stabilisiertem Hafnium, Calcium-stabilisiertem Hafnium und Magnesium-stabilisiertem Hafnium.

13. Verfahren gemäß einem der Ansprüche 1 bis 11, wobei die Wärmedämmbeschichtungszusammensetzung ein Yttrium-stabilisiertes Zirkoniumpulver aufweist.

## Revendications

1. Procédé de revêtement d'un article, comprenant :
l'application (10) d'une couche d'accrochage sur au moins une surface d'un article ;
l'application (12) sur ladite couche d'accrochage d'une composition de revêtement de barrière thermique comprenant une distribution de taille de particules de pas moins de 8 µm et pas plus de 88 µm ; et
le traitement thermique (14, 16) de ladite composition de revêtement de barrière thermique à une température comprise entre 1800 °F et 2200 °F (982 °C et 1204 °C) pendant 2 heures à 4 heures à une pression de 1.10⁻³ Torr à 1.10⁻⁶ Torr (133 à 0,13 mPa) pour former une couche de revêtement de barrière thermique comprenant une densité de fissuration de 1 fissure à 20 fissures par pouce linéaire (0,4 à 7,9 fissures par cm) dudit revêtement de barrière thermique, une porosité moyenne comprise entre pas plus de 5 pour cent et 0 pour cent, et une densité moyenne comprise entre 95 pour cent et 100 pour cent ; et dans lequel
l'application de ladite composition de revêtement de barrière thermique comprend un procédé choisi dans le groupe constitué par les procédés de projection au plasma, les procédés de projection au plasma à basse pression, les procédés de projection au plasma atmosphérique, les procédés de pulvérisation, les procédés à arc cathodique, les procédés de dépôt physique en phase vapeur par faisceau d'électrons, les procédés de projection au plasma à haute vitesse, les procédés de combustion, les procédés de projection au fil, les procédés de rechargement par faisceau laser et les procédés de rechargement par faisceau d'électrons, ou une combinaison comprenant l'un au moins de ces procédés.

2. Procédé selon la revendication 1, dans lequel l'étape de traitement thermique (14) comprend le traitement thermique de ladite composition de revêtement de barrière thermique sous ledit vide à une température de 2175 °F (1191 °C) pendant 2 heures.

3. Procédé selon la revendication 1, dans lequel l'étape de traitement thermique (14) comprend le traitement thermique de ladite composition de revêtement de barrière thermique sous ledit vide à une température de 2050 °F (1121 °C) pendant 2 heures.

4. Procédé selon la revendication 1, dans lequel l'étape de traitement thermique (14) comprend le traitement thermique de ladite composition de revêtement de barrière thermique sous ledit vide à une température de 1800 °F (982 °C) pendant 4 heures.

5. Procédé selon la revendication 1, dans lequel l'étape de traitement thermique (14) comprend le traitement thermique de ladite composition de revêtement de barrière thermique sous ledit vide à une température de 2100 °F (1149 °C) pendant 4 heures.

6. Procédé selon l'une quelconque des revendications précédentes, dans lequel l'étape d'application (10) de ladite couche d'accrochage comprend un procédé choisi dans le groupe constitué par les procédés de diffusion, les procédés de projection au plasma, les procédés de projection au plasma à basse pression, les procédés de projection au plasma atmosphérique, les procédés de pulvérisation, les procédés à arc cathodique, les procédés de dépôt physique en phase vapeur, les procédés de dépôt physique en phase vapeur par faisceau d'électrons, les procédés de projection au plasma à haute vitesse, les procédés de combustion, les procédés de projection au fil, les procédés de rechargement par faisceau laser et les procédés de rechargement par faisceau d'électrons.

7. Procédé selon l'une quelconque des revendications précédentes, dans lequel l'étape d'application (12) de ladite composition de revêtement de barrière thermique comprend l'application de ladite composition de revêtement de barrière thermique à l'aide d'un procédé de projection au plasma,

8. Procédé selon la revendication 7, dans lequel l'étape d'application (12) de ladite composition de revêtement de barrière thermique comprend l'utilisation d'un gaz d'arc comprenant de l'hélium et de l'argon présents dans un rapport de 3:1 à 1:3.

9. Procédé selon la revendication 7 ou 8, dans lequel l'étape d'application de ladite composition de revêtement de barrière thermique comprend l'utilisation d'un pistolet de projection au plasma à injection de poudre interne.

10. Procédé selon la revendication 9, comprenant en outre le fonctionnement dudit pistolet de projection au plasma à injection de poudre interne à un courant compris entre 600 et 1000 A.

11. Procédé selon la revendication 9 ou 10, comprenant en outre le fonctionnement dudit pistolet de projection au plasma à injection de poudre interne à une distance de 2 pouces à 8 pouces (5,1 à 20,3 cm) de ladite au moins une surface dudit article.

12. Procédé selon l'une quelconque des revendications précédentes, dans lequel ladite composition de revêtement de barrière thermique comprend un matériau céramique en poudre choisi dans le groupe constitué par la zircone stabilisée à l'oxyde d'yttrium, la zircone stabilisée à l'oxyde de calcium, la zircone stabilisée à la magnésie, l'oxyde de hafnium stabilisé à l'oxyde d'yttrium, l'oxyde de hafnium stabilisé à l'oxyde de calcium et l'oxyde de hafnium stabilisé à la magnésie.

13. procédé selon l'une quelconque des revendications 1 à 11, dans lequel ladite composition de revêtement de barrière thermique comprend une poudre de zircone stabilisée à l'oxyde d'yttrium.
